

## UNITED STATES PATENT OFFICE

GEORGE HOLLAND ELLIS AND HENRY CHARLES OLPIN, OF SPONDON, NEAR DERBY, ENGLAND, ASSIGNEES TO CELANESE CORPORATION OF AMERICA, A CORPORATION OF DELAWARE

## TREATMENT OF CELLULOSE DERIVATIVES

No Drawing. Application filed September 29, 1928, Serial No. 309,350, and in Great Britain November 15, 1927.

This invention relates primarily to the weighting of fibres, yarns, woven, knitted or other fabrics or other products made with or containing cellulose acetate or other organic acid esters of cellulose, for example, cellulose 5 formate, propionate or butyrate, or made with or containing cellulose ethers, for example, methyl, ethyl or benzyl cellulose or the corresponding condensation products of cellulose and glycols or other polyhydric alcohols. All such cellulose derivatives are hereinafter, for the sake of brevity, referred to as organic substitution derivatives of cellulose.

15 Prior U. S. application S. No. 57,956 filed 22nd September, 1925, describes the loading of such materials or products by treatment with a metallic salt solution, for example, stannic chloride, and subsequent fixing of the 20 metal in insoluble form, for instance by treatment with a phosphate, silicate or tannic acid and further describes how the weighting may be assisted by the use of swelling agents. Later applications have described how the 25 weighting treatment may be assisted by the use of organic swelling agents.

We have now found that the weighting with stannic chloride or other metallic salts may be very greatly assisted by the use of 30 organic salts, which exert a gelling or swelling action upon the cellulose derivatives.

In general such salts are metallic salts of high solubility in water. Zinc salts of high solubility, and particularly, zinc chloride, are 35 found to be especially useful.

Salts which form double salts with the weighting agent or agents used, as for example sodium or calcium chloride with stannic chloride, should be avoided.

40 One advantage of the use of these inorganic gelling salts is that they enable the treatment to be carried out at lower temperatures to obtain any given degree of weighting. This is especially useful in treating mixed materials containing natural silk in addition to the cellulose derivatives.

Textile materials treated in accordance with the present invention are found to have improved handle or feel, improved dyeing properties, and increased resistance to heat

treatments such as ironing (particularly noticeable with materials made from or containing dry-spun cellulose acetate filaments), and the tendency of circular knitted fabrics to ladder, of warp-knitted fabrics to split and of woven fabrics to slip is considerably reduced and may even be eliminated.

The process of the present invention, i. e. the use as assistants of inorganic salts which exert a gelling action upon the cellulose derivatives, is further found to be applicable with advantage to the mordanting of materials made with or containing cellulose acetate or other organic substitution derivatives of cellulose. Thus for example, the materials may be mordanted with iron, chromium, aluminium or tin with the assistance of the said inorganic gelling salts.

In carrying out the process of the present invention the material made of or containing the cellulose acetate etc. may be treated in hank, fabric or other form with a solution of the desired weighting or mordanting metal, e. g. a solution of stannic chloride, in the presence of the salt favourable to the gelation of the cellulose derivatives, for example zinc chloride.

The conditions and concentrations of the weighting (or mordanting) and gelling agents may vary considerably according to 80 the amount of weighting (or mordanting) required, it being found in particular that the factors of time, temperature and relative and total concentrations of the weighting (or mordanting) salt and the gelling salt govern 85 the amount of metal absorbed. The concentrations and other conditions should not be such as to dissolve or peptize the cellulose derivative or otherwise to damage the permanence, strength, lustre or other characteristics 90 of the materials treated.

Any suitable manipulative method may be used for the purpose of the invention. For example, yarns in hank form or fabrics in a suitably folded form may be treated by a 95 simple immersion method by hand in an open vat. Alternatively, a continuous method, particularly suitable for piece goods, may be employed, the material being passed through the solution or solutions and then evenly 100

squeezed or otherwise extracted. The goods thus treated are preferably allowed to lie for some time to allow maximum absorption to take place.

- 5 In general, higher temperatures and/or higher concentrations will be required in the continuous method in order to obtain the same amount of weighting or mordanting as in the immersion method, since the latter method 10 permits of contact with the liquor during a longer period.

After the absorption of the weighting or mordanting metal the goods are preferably washed off and may then be subjected to any 15 suitable after-treatments. For example they may be treated with phosphate or silicate or other suitable precipitant for the absorbed metal, or, if desired, precipitation may be effected by a simple washing, a little lime or 20 other alkali being present in the washing water.

Heavier weightings may be obtained by repeating one or more times the treatment with the weighting metal salts, the subsequent 25 treatments either preceding or following the treatment with the precipitant.

Materials mordanted according to the present invention may afterwards be dyed with any suitable mordant dyestuffs, natural 30 or artificial.

The following examples are intended to be purely illustrative of the invention and not limitative of its scope:—

#### 35 Example 1

A weighting liquor is made up containing 355 grams stannic chloride commercial crystals and 355 grams zinc chloride per litre of solution at 25° C. Cellulose acetate woven 40 fabric, previously scoured and dried, is entered, and allowed to steep for 1 hour. The goods are then lifted carefully, and washed well till the fabric is free from acidity. A treatment of  $\frac{1}{2}$  hour is then given in a 10% 45 disodium hydrogen phosphate solution at 60° C. after which the goods are rinsed, given a light soaping in a  $\frac{1}{4}\%$  soap solution at 45° C. for  $\frac{1}{4}$  hour rinsed again, and dried or otherwise treated as requisite. The goods 50 thus treated show an increase in weight of 7.5-10% whereas omission of the zinc chloride leads to a weighting of only about 2.5%.

#### 55 Example 2

A mordanting liquor is made up containing 300 grams of ferric chloride and 300 grams of zinc chloride per litre at 30° C. Cellulose acetate woven fabric, previously 60 scoured and dried, is entered, and allowed to steep for one hour. The goods are then lifted carefully and washed well in several changes of cold water until the washings are free from acidity, and any trace of iron salt, and 65 then lifted, and dried or otherwise treated as

requisite. They may be dyed with any mordant dyestuffs, natural or artificial.

Materials made with or containing other organic substitution derivatives of cellulose, for example cellulose formate, propionate or 70 butyrate or methyl or ethyl cellulose, may be weighted or mordanted in a similar manner.

What we claim and desire to secure by Letters Patent is:—

1. In a process for weighting materials comprising organic derivatives of cellulose with tin compounds, the step of treating the materials with a solution containing stannic chloride and zinc chloride in such concentration as to swell the organic derivative of cellulose. 75

2. In a process for weighting materials comprising cellulose acetate with tin compounds, the step of treating the materials with a solution containing stannic chloride and zinc chloride in such concentration as to swell the cellulose acetate. 85

3. In a process for weighting materials comprising organic derivatives of cellulose with tin compounds, the step of treating the materials with a solution containing a tin salt and a zinc salt in such concentration as to swell the organic derivative of cellulose. 90

4. In a process for weighting materials comprising cellulose acetate with tin compounds, the step of treating the materials with a solution containing a tin salt and a zinc salt in such concentration as to swell the cellulose acetate. 95

In testimony whereof, we have hereunto 100 subscribed our names.

GEORGE HOLLAND ELLIS.  
HENRY CHARLES OLPIN.

105

110

115

125

130